



US007820310B2

(12) **United States Patent**  
**Björmander**

(10) **Patent No.:** **US 7,820,310 B2**  
(45) **Date of Patent:** **Oct. 26, 2010**

(54) **COATED CUTTING TOOL INSERT**

(75) Inventor: **Carl Björmander**, Spågna (SE)

(73) Assignee: **Sandvik Intellectual Property AB**,  
Sandviken (SE)

(\*) Notice: Subject to any disclaimer, the term of this  
patent is extended or adjusted under 35  
U.S.C. 154(b) by 0 days.

(21) Appl. No.: **12/320,578**

(22) Filed: **Jan. 29, 2009**

(65) **Prior Publication Data**

US 2009/0136728 A1 May 28, 2009

**Related U.S. Application Data**

(62) Division of application No. 11/403,206, filed on Apr.  
13, 2006, now Pat. No. 7,531,213.

(30) **Foreign Application Priority Data**

Apr. 18, 2005 (SE) .....

(51) **Int. Cl.**

**B32B 9/00** (2006.01)

(52) **U.S. Cl.** .....

**428/701**; 51/307; 51/309;  
428/697; 428/698; 428/702; 428/216; 428/336

(58) **Field of Classification Search** .....

51/307,  
51/309; 428/697, 698, 699, 701, 702, 704,  
428/216, 336

See application file for complete search history.

(56) **References Cited**

U.S. PATENT DOCUMENTS

|                |         |                     |
|----------------|---------|---------------------|
| 4,150,195 A    | 4/1979  | Tobioka et al.      |
| 4,714,660 A    | 12/1987 | Gates, Jr.          |
| 5,654,035 A    | 8/1997  | Ljungberg et al.    |
| 5,770,261 A    | 6/1998  | Nakamura et al.     |
| 5,800,868 A    | 9/1998  | Lenander et al.     |
| 5,861,210 A    | 1/1999  | Lenander et al.     |
| 6,071,601 A *  | 6/2000  | Oshika et al. ..... |
| 6,426,137 B1   | 7/2002  | Oshika et al.       |
| 6,733,874 B2 * | 5/2004  | Ueda et al. .....   |

|                 |         |                         |
|-----------------|---------|-------------------------|
| 7,153,562 B2    | 12/2006 | Rodmar et al.           |
| 7,276,301 B2    | 10/2007 | Tsushima et al.         |
| 7,326,461 B2 *  | 2/2008  | Sottke et al. .....     |
| 7,531,213 B2 *  | 5/2009  | Björmander .....        |
| 7,597,951 B2 *  | 10/2009 | Björmander et al. ..... |
| 2002/0187370 A1 | 12/2002 | Yamagata et al.         |
| 2004/0224160 A1 | 11/2004 | Ueda et al.             |
| 2005/0260432 A1 | 11/2005 | Sottke et al.           |
| 2007/0298232 A1 | 12/2007 | McNerny et al.          |

FOREIGN PATENT DOCUMENTS

|    |              |         |
|----|--------------|---------|
| EP | 0 693 574 B2 | 4/2001  |
| EP | 0 878 563 B1 | 10/2001 |
| EP | 1 455 003 A2 | 9/2004  |
| EP | 1 705 263 A1 | 9/2006  |
| EP | 1 717 348 A2 | 11/2006 |
| JP | 11-152570    | 6/1999  |
| JP | 2004-1888501 | 7/2004  |
| WO | 02/04156     | 1/2002  |

OTHER PUBLICATIONS

Sahin, Y., "The Effects of Various Multilayer Ceramic Coatings on the Wear of Carbide Cutting Tools When Machining Metal Matrix Composites", *Surface and Coatings Technology*, vol. 199, Issue 1, Sep. 1, 2005, pp. 112-117.

\* cited by examiner

Primary Examiner—Archene Turner

(74) Attorney, Agent, or Firm—Drinker Biddle & Reath LLP

(57) **ABSTRACT**

A method for making a coated cutting tool insert by depositing by CVD, onto a cemented carbide, titanium based or ceramic substrate a hard layer system, having a total thickness of from about 2 to about 50  $\mu$ m, comprising at least one layer selected from titanium carbide, titanium nitride, titanium carbonitride, titanium carboxide and aluminum oxide, and an outer, from about 1 to about 15  $\mu$ m thick, aluminum oxide layer or  $(Al_2O_3+ZrO_2)^*N$  multilayer, a penultimate outermost layer of  $TiO_x$ , where x ranges from about 1 to about 2, and an outermost, from about 0.3 to about 2  $\mu$ m thick,  $TiC_xN_yO_z$  layer, where  $x+y+z=1$ ,  $x \geq 0$ ,  $y \geq 0$ , and  $z \geq 0$ , followed by a post-treatment removing at least said outermost layer on the edge-line and on the rake face.

**12 Claims, 3 Drawing Sheets**



Fig. 1A



Fig. 1B



Fig. 1C



Fig. 2A



Fig. 2B



Fig. 2C



**Fig. 3**

**1**  
**COATED CUTTING TOOL INSERT**

RELATED APPLICATION DATA

This application is a divisional application of U.S. Application Ser. No. 11/403,206, filed Apr. 13, 2006, claims priority under 35 U.S.C. §119 and/or §365 to Swedish Application No. 0500858-6, filed Apr. 18, 2005, the entire contents of each of these applications are incorporated herein by reference.

BACKGROUND

The present invention relates to a coated cutting tool, suitable for chip forming machining of metals, and a method for producing the same. According to the present invention, there is provided a reliable method for removing coating layers on selected faces of a cutting insert during coating post-treatment.

Modern high productivity chip forming machining of metals requires reliable tools with excellent wear properties. This is achieved by employing a cemented carbide tool body coated with a wear resistant coating, of single layer or multilayer type, most commonly comprising wear layers of TiC, TiN, TiCN and Al<sub>2</sub>O<sub>3</sub>. For depositing the different layers onto the cemented carbide body, CVD, PVD, or similar coating techniques are used.

EP-A-693574 describes how different parts of a tool are subject to different types of wear during a machining operation. Since the various coating layers have different abilities to withstand the different types of wear, it is suggested to have an outermost Al<sub>2</sub>O<sub>3</sub> layer on the rake face, because of its ability to withstand diffusion type wear, and on the clearance side it is suggested to have an outermost MeC<sub>x</sub>N<sub>y</sub>O<sub>z</sub> type layer, where Me is a metal selected from groups IVB, VB, VIB of the periodic table, because of its high resistance to flank wear. A top layer of TiC<sub>x</sub>N<sub>y</sub>O<sub>z</sub> or, in particular, a goldish TiN, ZrN or HfN top layer also makes it easy to differentiate between a used and an unused cutting edge by the naked eye. Hence, the TiC<sub>x</sub>N<sub>y</sub>O<sub>z</sub> layer is mechanically removed from either only the edge line or from both the rake face and the edge line to expose the Al<sub>2</sub>O<sub>3</sub> layer. Normally this is done by a post-treatment such as blasting or brushing of the coated inserts.

During the post-treatment, it is important not to reduce the Al<sub>2</sub>O<sub>3</sub> layer thickness along the edge line. The method must therefore be so gentle that only the top TiC<sub>x</sub>N<sub>y</sub>O<sub>z</sub> layer is removed, leaving the Al<sub>2</sub>O<sub>3</sub> at the edge line as untouched as possible. However, the described post-treatment method is unreliable as residues of TiC<sub>x</sub>N<sub>y</sub>O<sub>z</sub> occasionally appear on the Al<sub>2</sub>O<sub>3</sub> surface after blasting process. TiC<sub>x</sub>N<sub>y</sub>O<sub>z</sub> residues on the Al<sub>2</sub>O<sub>3</sub> surface reduce the flaking resistance, due to welding of TiC<sub>x</sub>N<sub>y</sub>O<sub>z</sub> to the work piece at the cutting edge resulting in coating withdrawal and a lower lifetime of the insert. A second effect of these residues after blasting is the discoloration, visible to the naked eye, of the Al<sub>2</sub>O<sub>3</sub> surface. In production, blasting is usually repeated or modified in order to remove residual TiC<sub>x</sub>N<sub>y</sub>O<sub>z</sub>, but this often results in damage, such as flaking of the coating at the cutting edge line. It is therefore important to find a solution to this problem, especially for thin Al<sub>2</sub>O<sub>3</sub> coatings, where usually lower blasting pressures are used in order not to damage the coating at the cutting edge, thus being subject to a higher risk of having TiC<sub>x</sub>N<sub>y</sub>O<sub>z</sub> residues after the blasting process.

In U.S. Pat. No. 6,426,137, a titanium oxide layer is utilized in order to reduce smearing onto the cutting edge. In this case the titanium oxide layer is fully covering the Al<sub>2</sub>O<sub>3</sub>

surface, acting as the top layer with a thickness of 0.1-3 µm. In another embodiment the titanium oxide layer is coated with a TiN layer.

5     OBJECTS AND SUMMARY OF THE INTENTION

It is an object of the present invention to solve the problem of residual TiC<sub>x</sub>N<sub>y</sub>O<sub>z</sub> on the post-treated edge line and rake face.

10    In accordance with the invention there is provided a method for making a coated cutting tool insert having an upper face (rake face), an opposite face and at least one clearance face intersecting said upper and opposite faces to define cutting edges comprising depositing by CVD, onto a cemented carbide, titanium based or ceramic substrate  
15    a hard layer system, having a total thickness of about from about 2 to about 50 µm, comprising at least one layer selected from titanium carbide, titanium nitride, titanium carbonitride, titanium carboxide and aluminum oxide, and an outer, from about 1 to about 15 µm thick, aluminum oxide layer or (Al<sub>2</sub>O<sub>3</sub>+ZrO<sub>2</sub>)<sup>\*N</sup> multilayer, a penultimate outermost layer of TiO<sub>x</sub>, where x ranges from about 1 to about 2 and  
20    an outermost, from about 0.3 to about 2 µm thick, TiC<sub>x</sub>-N<sub>y</sub>O<sub>z</sub> layer, where x+y+z=1, x≥0, y≥0, and z≥0,  
25    by a post-treatment removing at least said outermost layer on the edge-line and on the rake face.

30     BRIEF DESCRIPTION OF THE FIGURES

35    FIGS. 1A-1C are light microscope micrographs showing in 200X, the outermost Al<sub>2</sub>O<sub>3</sub> layer of inserts according to the present invention, with various amounts of titanium nitride residues after the blasting process, in which in FIG. 1A  
40    A—TiN residues, and  
45    B—Al<sub>2</sub>O<sub>3</sub>.

FIGS. 2A-2C are scanning electron microscope micrographs showing in 500X, the outermost Al<sub>2</sub>O<sub>3</sub> layer of inserts according to the present invention, with various amounts of titanium oxide residues after the blasting process, in which in FIG. 2A  
45    A—Ti<sub>2</sub>O<sub>3</sub> residues, and  
50    B—Al<sub>2</sub>O<sub>3</sub>.

FIG. 3 is a light microscope micrograph showing in 200X, the outermost Al<sub>2</sub>O<sub>3</sub> layer of an insert edge according to the prior art, with titanium nitride residues after the blasting process, in which  
55    A—TiN residues, and  
60    B—Al<sub>2</sub>O<sub>3</sub>.

55     DETAILED DESCRIPTION OF THE PREFERRED  
60     EMBODIMENTS OF THE INVENTION

According to the present invention, there is now provided a method of making a coated cutting tool insert, having an upper face (rake face), an opposite face and at least one clearance face intersecting said upper and opposite faces to define cutting edges, comprising depositing onto a cemented carbide, titanium based or ceramic substrate, using known CVD methods

65    a hard layer system, having a total thickness of from about 2 to about 50 µm, comprising least one layer selected from titanium carbide, titanium nitride, titanium carbonitride, titanium carboxide and aluminum oxide, and an outer, from about 1 to about 15 µm thick, aluminum oxide layer or (Al<sub>2</sub>O<sub>3</sub>+ZrO<sub>2</sub>)<sup>\*N</sup> multilayer,

a penultimate outermost layer of  $\text{TiO}_x$ , where  $x$  ranges from about 1 to about 2, preferably from about 1.3 to about 1.9, having a thickness preferably from about 0.05 to about 3  $\mu\text{m}$ , most preferably from about 0.1 to about 1.0  $\mu\text{m}$ , and

an outermost, from about 0.3 to about 2  $\mu\text{m}$  thick,  $\text{TiC}_x\text{N}_y\text{O}_z$  layer, where  $x+y+z=1$ ,  $X \geq 0$ ,  $y \geq 0$ , and  $z \geq 0$ , preferably a single layer or multilayer of  $\text{TiN}$ ,  $\text{TiC}$  or  $\text{TiC}_x\text{N}_y$ , where  $x+y=1$ ,  $x \geq 0$  and  $y \geq 0$ ,

followed by a post-treatment, preferably blasting or brushing, removing at least said outermost layer on the edge-line and on the rake face. To ensure the performance of the insert and the absence of any discoloration due to  $\text{TiN}$  residues, it is preferred that said post-treatment also removes at least 50% of the  $\text{TiO}_x$  layer, in terms of surface coverage, i.e., preferably at least 50% of the outer layer surface of said hard layer system is exposed.

Using  $\text{TiO}_x$ , which has a hardness of about 20% of that of  $\text{Al}_2\text{O}_3$ , with the proposed thickness, the  $\text{TiC}_x\text{N}_y\text{O}_z$  layer is thus lifted up above the rough  $\text{Al}_2\text{O}_3$  surface, so that it can be fully removed by the blasting media.  $\text{TiO}_x$  is furthermore a transparent oxide, which means that any residues left on the  $\text{Al}_2\text{O}_3$  surface are not visible to the naked eye, as is the case with, e.g.,  $\text{TiN}$ .

The present invention also relates to a coated cutting tool insert having an upper face (rake face), an opposite face and at least one clearance face intersecting said upper and opposite faces to define cutting edges made of cemented carbide, titanium based carbonitride or ceramics. The insert is coated with a hard layer system, having a total thickness of from about 2 to about 50  $\mu\text{m}$ , comprising at least one layer selected from titanium carbide, titanium nitride, titanium carbonitride, titanium carboxide and aluminum oxide, and an outer, from about 1 to about 15  $\mu\text{m}$  thick, aluminum oxide, preferably fine grained of a grain size of from about 0.50 to about 3  $\mu\text{m}$ ,  $\alpha\text{-Al}_2\text{O}_3$ , layer or  $(\text{Al}_2\text{O}_3+\text{ZrO}_2)^*\text{N}$  multilayer, said hard layer system is provided with a  $\text{TiO}_x$  layer, where  $x$  ranges from about 1 to about 2, preferably from about 1.3 to about 1.9, with a thickness of preferably from about 0.05 to about 3  $\mu\text{m}$ , most preferably 0.1-1.0  $\mu\text{m}$ , said  $\text{TiO}_x$  layer being the outermost layer on the cutting edge line and rake face, and said  $\text{TiO}_x$  layer is on the clearance side provided with an outermost, 0.3-2  $\mu\text{m}$  thick,  $\text{TiC}_x\text{N}_y\text{O}_z$  layer, where  $x+y+z=1$ ,  $x \geq 0$ ,  $y \geq 0$ , and  $z \geq 0$ , preferably a single layer or multilayer of  $\text{TiN}$ ,  $\text{TiC}$  or  $\text{TiC}_x\text{N}_y$ , where  $x+y=1$ ,  $x \geq 0$  and  $y \geq 0$ .

The grain size of the  $\text{Al}_2\text{O}_3$  layer is determined from a SEM top view micrograph at 5,000 X magnification of the as deposited  $\text{Al}_2\text{O}_3$  layer surface. Drawing three straight lines in random directions, the average distances between grain boundaries along the lines, are taken as a measure of the grain size.

In a preferred embodiment said  $\text{TiO}_x$  layer on the edge-line and rake face covers less than 50% of the surface of said hard layer system.

The invention is additionally illustrated in connection with the following examples, which are to be considered as illustrative of the present invention. It should be understood, however, that the invention is not limited to the specific details of the examples.

#### EXAMPLE 1

A (invention): Cemented carbide cutting inserts CNMG 120408-PM with the composition 5.5 wt-% Co, 8.6 wt-% cubic carbides ( $\text{TiC}+\text{TaC}+\text{NbC}$ ) and balance WC were coated with CVD-technique according to the following sequence: 0.7  $\mu\text{m}$   $\text{TiN}$ , 4.0  $\mu\text{m}$   $\text{Ti}(\text{CN})$ , 5.0  $\mu\text{m}$   $\alpha\text{-Al}_2\text{O}_3$ , 0.7  $\mu\text{m}$  titanium oxide ( $\text{Ti}_2\text{O}_3$ ) and 0.7  $\mu\text{m}$   $\text{TiN}$ .

The  $\text{Ti}_2\text{O}_3$  layer was deposited by CVD technique, where the substrates to be coated were held at a temperature of 1010° C. and were brought in contact with a hydrogen carrier gas containing  $\text{TiCl}_4$ ,  $\text{CO}_2$  and  $\text{HCl}$ . The nucleation was started up in a sequence where the reactant gases  $\text{HCl}$  and  $\text{CO}_2$  entered the reactor first, in an  $\text{H}_2$  atmosphere, followed by the  $\text{TiCl}_4$ . The titanium oxide layer was deposited with a CVD process with the following process parameters:

| Gasflows (in %).<br>$T = 1010^\circ \text{C.}, P = 55 \text{ mbar.}$ |  | $\text{Ti}_2\text{O}_3$ |
|----------------------------------------------------------------------|--|-------------------------|
| $\text{H}_2$ (%)                                                     |  | 88.0                    |
| $\text{HCl}$ (%)                                                     |  | 7.6                     |
| $\text{CO}_2$ (%)                                                    |  | 2.1                     |
| $\text{TiCl}_4$ (%)                                                  |  | 2.3                     |
| Deposition Rate ( $\mu\text{m}/\text{hrs}$ )                         |  | 1.5                     |

The other layers were deposited by known CVD methods.

The coated inserts were post-treated by blasting at the different blasting pressures 1.8, 2.0 and 2.2 bar, using  $\text{Al}_2\text{O}_3$  grits.

B (prior art): Cemented carbide cutting inserts CNMG 120408-PM with the composition 5.5 wt-% Co, 8.6 wt-% cubic carbides ( $\text{TiC}+\text{TaC}+\text{NbC}$ ) and balance WC were coated with CVD-technique according to the following sequence: 0.7  $\mu\text{m}$   $\text{TiN}$ , 4.0  $\mu\text{m}$   $\text{Ti}(\text{CN})$ , 5.0  $\mu\text{m}$   $\alpha\text{-Al}_2\text{O}_3$  and 0.7  $\mu\text{m}$   $\text{TiN}$  by known CVD methods.

The coated inserts were post treated by blasting at 2.4 bar by using  $\text{Al}_2\text{O}_3$  grits.

Inserts of type A and B were studied in a light microscope (200X) to detect any  $\text{TiN}$  residues on the  $\text{Al}_2\text{O}_3$  surface and further in a scanning electron microscope (500X) to detect residues of  $\text{Ti}_2\text{O}_3$ . The amount of residual  $\text{Ti}_2\text{O}_3$  was determined using image analysis (Leica Quantimet 500). The results are summarized in the following table.

|                                           |                                                                                                                                                                                    |                                                                                                         |
|-------------------------------------------|------------------------------------------------------------------------------------------------------------------------------------------------------------------------------------|---------------------------------------------------------------------------------------------------------|
| Sample A, blasting at 1.8 bar (invention) | Some amount of $\text{TiN}$ residues on the $\text{Al}_2\text{O}_3$ -surface as observed by light microscope (FIG. 1A). Insert surface appear lightly discolored to the naked eye. | <75% of $\text{Al}_2\text{O}_3$ -surface covered by residual $\text{Ti}_2\text{O}_3$ (FIG. 2A).         |
| Sample A, blasting at 2.0 bar (invention) | <1% of $\text{Al}_2\text{O}_3$ -surface covered by residual $\text{TiN}$ (FIG. 1B). No discoloration of the insert                                                                 | <50% of $\text{Al}_2\text{O}_3$ -surface covered by residual $\text{Ti}_2\text{O}_3$ surface. (FIG. 2B) |

-continued

|                                            |                                                                                                                                                                          |                                                                                                                |
|--------------------------------------------|--------------------------------------------------------------------------------------------------------------------------------------------------------------------------|----------------------------------------------------------------------------------------------------------------|
| Sample A, blasting at 2.2 bar, (invention) | No residues of TiN (FIG. 1C). No discoloration of the insert surface.                                                                                                    | <30% of Al <sub>2</sub> O <sub>3</sub> -surface covered by residual Ti <sub>2</sub> O <sub>3</sub> . (FIG. 2C) |
| Sample B, blasting at 2.4 bar (prior art)  | Large amount of TiN residues on the Al <sub>2</sub> O <sub>3</sub> -surface as observed by light microscope (FIG. 2). Insert surface appear discolored to the naked eye. | —                                                                                                              |

Although the present invention has been described in connection with preferred embodiments thereof, it will be appreciated by those skilled in the art that additions, deletions, modifications, and substitutions not specifically described may be made without departing from the spirit and scope of the inventions as defined in the appended claims.

The invention claimed is:

1. A coated cutting tool insert having an upper face (rake face), an opposite face, and at least one clearance face intersecting said upper and opposite faces to define cutting edges, wherein said cutting tool insert is made of a cemented carbide or a ceramic substrate, said cutting tool coated with a hard layer system having a total thickness of from about 2 to about 50  $\mu\text{m}$  and comprising

at least one layer selected from titanium carbide, titanium nitride, titanium carbonitride, titanium carboide, and aluminum oxide;

an outer layer of an aluminum oxide, said outer layer being about 1 to about 15  $\mu\text{m}$  thick;

an outermost TiO<sub>x</sub> layer on the cutting edges and rake face, where x ranges from about 1 to about 2;

a penultimate outermost TiO<sub>x</sub> layer on the clearance side; and

an outermost TiC<sub>x</sub>N<sub>y</sub>O<sub>z</sub> layer on the clearance side, wherein x+y+z=1, x $\geq$ 0, y $\geq$ 0, and z $\geq$ 0 and said outermost TiC<sub>x</sub>N<sub>y</sub>O<sub>z</sub> layer is from about 0.3 to about 2  $\mu\text{m}$  thick.

2. The cutting tool insert of claim 1 wherein said TiO<sub>x</sub> layer on the cutting edges and rake face covers less than 50% of said edges and rake face.

3. The cutting tool insert of claim 1 wherein said outermost or said penultimate outermost TiO<sub>x</sub> layer has a thickness of from about 0.05 to about 3  $\mu\text{m}$ .

4. The cutting tool insert of claim 1 wherein said TiC<sub>x</sub>N<sub>y</sub>O<sub>z</sub> layer is a single or multilayer of TiN, TiC or TiC<sub>x</sub>N<sub>y</sub> where x+y=1, x $\geq$ 0 and y $\geq$ 0.

5. The cutting tool insert of claim 1 wherein said outer layer of an aluminum oxide is a fine grained  $\alpha$ -Al<sub>2</sub>O<sub>3</sub> layer.

6. The coated cutting tool of claim 1, wherein said outer layer of aluminum oxide is an (Al<sub>2</sub>O<sub>3</sub>+ZrO<sub>2</sub>)<sup>\*</sup>N multilayer.

7. A coated cutting tool insert having an upper face (rake face), an opposite face, and at least one clearance face intersecting said upper and opposite faces to define cutting edges, wherein said cutting tool insert is made of a titanium based carbonitride, said cutting tool coated with a hard layer system having a total thickness of from about 2 to about 50  $\mu\text{m}$  and comprising

at least one layer selected from titanium carbide, titanium nitride, titanium carbonitride, titanium carboide, and aluminum oxide;

an outer layer of an aluminum oxide, said outer layer being about 1 to about 15  $\mu\text{m}$  thick;

an outermost TiO<sub>x</sub> layer on the cutting edges and rake face, where x ranges from about 1 to about 2;

a penultimate outermost TiO<sub>x</sub> layer on the clearance side; and

an outermost TiC<sub>x</sub>N<sub>y</sub>O<sub>z</sub> layer on the clearance side, wherein x+y+z=1, x $\geq$ 0, y $\geq$ 0, and z $\geq$ 0 and said outermost TiC<sub>x</sub>N<sub>y</sub>O<sub>z</sub> layer is from about 0.3 to about 2  $\mu\text{m}$  thick.

8. The cutting tool insert of claim 7 wherein said TiO<sub>x</sub> layer on the cutting edges and rake face covers less than 50% of said edges and rake face.

9. The cutting tool insert of claim 7 wherein said outermost or said penultimate outermost TiO<sub>x</sub> layer has a thickness of from about 0.05 to about 3  $\mu\text{m}$ .

10. The cutting tool insert of claim 7 wherein said TiC<sub>x</sub>-N<sub>y</sub>O<sub>z</sub> layer is a single or multilayer of TiN, TiC or TiC<sub>x</sub>N<sub>y</sub> where x+y=1, x $\geq$ 0 and y $\geq$ 0.

11. The cutting tool insert of claim 7 wherein said outer layer of an aluminum oxide is a fine grained  $\alpha$ -Al<sub>2</sub>O<sub>3</sub> layer.

12. The coated cutting tool of claim 7, wherein said outer layer of aluminum oxide is an (Al<sub>2</sub>O<sub>3</sub>+ZrO<sub>2</sub>)<sup>\*</sup>N multilayer.

\* \* \* \* \*